

March 13, 1945.

B. BANNISTER

2,371,125

## METHOD OF MAKING GUN BARREL FORGINGS

Filed Jan. 16, 1942

2 Sheets-Sheet 1

FIG. 1.



FIG. 2.



*Inventor:*  
BRYANT BANNISTER,  
by: *John E. Jackson*  
*his Attorney.*

March 13, 1945.

B. BANNISTER

2,371,125

METHOD OF MAKING GUN BARREL FORGINGS

Filed Jan. 16, 1942

2 Sheets-Sheet 2



FIG. 5.



FIG. 6.



FIG. 7.



FIG. 3.

Inventor:

BYRANT BANNISTER,  
by: *John E. Jackson*  
his Attorney.

## UNITED STATES PATENT OFFICE

2,371,125

## METHOD OF MAKING GUN BARREL FORGINGS

Bryant Bannister, Mount Lebanon, Pa., assignor  
to National Tube Company, a corporation of  
New Jersey

Application January 16, 1942, Serial No. 427,075

3 Claims. (Cl. 80—62)

This invention relates to the manufacture of gun barrels, and more particularly to those which in the past have to a large extent been formed by forging steel ingots in one or more operations into stock which can be turned and bored to the final dimensions. For guns of smaller size, centrifugal casting has been resorted to in order to eliminate a considerable portion of machine work involved in boring which is required where solid stock is employed. However, since a centrifugal casting cannot be tapered on the outside, this taper must be obtained by a machining operation. Machine work is expensive and slow and in times of national emergency, reduction in the extent thereof is very essential.

The stresses to which a gun barrel is subjected in service are so severe that the strength of material of which it is made must be high in all directions. To determine this strength, tests are made on specimens taken in both a longitudinal and transverse direction with respect to the axis of the barrel. Generally, the greatest strength is shown in the direction of metal flow during the forming or forging operation, as this flow orients the shear planes in the direction of flow; thus the strength transversely to the direction of flow is at a minimum. Since a gun barrel forging originates from a chunky ingot, the greatest flow of metal occurs lengthwise of the barrel; consequently the greatest strength is in this same direction. It has been proposed to reduce this disparity in strength by twisting the forging or casting while at an elevated temperature, to orientate the lines of weakness in a helical direction, thereby reducing the longitudinal and increasing the transverse strength. This twisting is in the nature of a separate operation, whereas in the practice of my invention it can be accomplished automatically as a part of the forming operation.

Conventional forging and centrifugal casting are inherently slow operations, necessitating the employment of great numbers of units and man power to produce the huge quantity of gun barrels required by a national emergency, whereas my method is capable of producing forgings at a tremendously greater rate per producing unit, the labor involved being correspondingly reduced.

It has long been known that the soundness and homogeneity of an ingot is greatly influenced by its contour and that the round corrugated design produces the best castings. Fortunately this type of ingot lends itself extremely well to my method of forging, which is in effect a rotary

blooming operation wherein the ingot is rotated and advanced helically between rolls which may be profiled to work the metal at the most desirable rate as the cross section is reduced, thereby maintaining the metal being worked in compression, and also, since the ingot is simultaneously pierced, the flow of metal proceeds both from the outside and the inside. By proper selection of ingot size with respect to the desired product, an exceptionally uniform, concentric and sound forging results. It has been found that in seamless tubular products which require exceptional quality of inside surface the above relationship is important to avoid surface imperfections which arise from segregations which are naturally located near the center of the ingot from which the seamless product is fabricated. In the case of gun barrel forgings, this undesirable material must be concentrated entirely within the surplus metal which is to be machined out in finishing the forging. This is easily provided for by first producing clean steel followed by proper teeming into ingot molds of the correct size and design.

25 It is among the objects of the present invention:

To provide a method of manufacturing gun barrel forgings according to which the shear planes in the metal thereof are orientated to a desired and controlled degree during an operation which forms the hollow workpiece;

30 To provide a method of manufacture according to which the transverse and longitudinal strength of the forging can be controlled to provide a uniform factor of safety in all directions when the gun is fired;

35 To so work the metal of the forging during the forming operation that at all times it is subjected only to compressive stresses, thereby producing a pressure forging wherein the metal is worked throughout its mass;

40 To provide a method of the class described which has great productivity and requires a minimum of man hours of labor per forging produced.

45 The foregoing and other objects will become more apparent after referring to the following specification and drawings wherein suitable apparatus for performing the method of my invention is disclosed, in which:

50 Figure 1 is a plan view of apparatus suitable for performing the method of the present invention.

Figure 2 is a side elevation partly in section.

55 Figure 3 shows a typical round corrugated ingot.

Figure 4 is a view showing the blooming and piercing operation being performed on an ingot.

Figure 5 shows the hollow forging after the above operation.

Figure 6 is a view showing a workpiece being reduced to final form between the rolls and the mandrel.

Figure 7 is a longitudinal section of the article produced by the method of the invention.

Referring more particularly to the drawings, the numeral 3 designates a pair of metal-working rolls disposed so as to helically advance a workpiece A over an interiorly disposed mandrel B. The rolls 3 are driven by motors 4 through shafts 5 and slip couplings 6. The shafts 5 are mounted in housings 7 which are slidably carried by bases 8. Also mounted on the bases 8, and at the rearward end thereof, are screw-nuts 10 engaging screws 11 which are secured to the housings 7. Screws 11 are connected by worm gears 12, shafts 13 and 14, gears 15 and speed reducer 16 to suitable motive power, such as a reversible electric motor 17, and it is seen that actuation thereof will move the rolls to enlarge or decrease the pass formed thereby.

Disposed adjacent the pass formed by the rolls 3, and intermediate thereof, are guides 20 which are pivotally mounted as at 21 and have grooved guiding surfaces 22, the grooves being of varying diameter and longitudinally curved on an arc having its focus offset with respect to the pivotal axis of the said guides. A frame, or housing 7<sup>a</sup> is disposed between and adjacent the housings 7 which carry the shafts 5 for the rolls 3. Mounted on this housing 7<sup>a</sup> are interior screw-nuts 23 having worm gear exteriors 24. Shafts 25 are connected to the guides 20 and have screw-threaded ends 26 disposed in the screw-nuts 23. A shaft 27 carries worms 28 which are in mesh with the gears 24, and this shaft is connected through a speed reducer 30 to a reversible motor or other source of power. Accordingly it is seen that operation thereof will move the guides 20 to enlarge or diminish the pass defined thereby.

In producing gun barrels by my method, it is possible to produce those of small caliber in one operation wherein the piercing and tapering is accomplished in one pass through the mill. In such cases it is also permissible to use a rolled round billet instead of an ingot, but for larger bore guns the method should employ at least two operations.

Where two operations are employed, the first may be either a simple piercing (wherein the solid ingot is reduced in diameter and simultaneously pierced, thereby producing a cylindrical hollow forging as shown in Figure 5), or the forging may be slightly tapered externally with a uniform bore. In the first instance, the forming rolls and guides remain a constant distance from the axis of the pass. In the second instance, the forming rolls and guides change distance from the axis of the pass during the rolling operation. The second operation (that of tapering the outside but maintaining the bore uniform) is carried out with a cylindrical mandrel inside the workpiece and with the rolls and guides varying in distance from the mill axis. This movement is controlled as hereinbefore described.

For very large bore guns, where large reductions are involved, a third operation similar to the second may be required.

During the initial piercing and subsequent operations, the forming rolls may be proportioned to produce a twist of the desired direction and extent to the workpiece or they may be so designed that no twist is produced. If a twist in the direction of rotation is desired, the roll speed at the "gorge" (or end of the reducing section of the pass) must be relatively faster than the speed at the beginning of rolling. Stated in another way, the roll must tend to rotate the billet a greater number of revolutions per unit of time at the gorge than it does at the inlet end of the pass. If a twist is desired opposite the direction of rotation, the reverse relationship must exist except that it has been found that the gorge roll speed can tend to rotate the billet faster than the roll does at the inlet without producing any twist. The twist in a gun barrel forging should be in a direction opposite the helical direction of the bore rifling to be machined into the barrel. Roll proportions may be such that substantially all twist can be imparted during the piercing operation, or in subsequent operations, or both.

While I have shown and described several specific embodiments of the present invention, it will be seen that I do not wish to be limited exactly thereto, since various modifications may be made without departing from the scope of the invention as defined in the appended claims.

I claim:

1. In the manufacture of gunbarrel forgings, the method which includes the steps of helically rolling a heated metallic workpiece over a mandrel to reduce the outside diameter thereof and to simultaneously pierce the same to provide a cylindrical forging having a bore of substantially the diameter desired in the finished article throughout the length thereof, then passing the workpiece over a mandrel between opposed, spaced-apart rolls whereby the workpiece is helically rolled and tapered by varying the distance between the rolls while maintaining the bore substantially uniform and maintaining the portion of the workpiece being worked under compression thereby producing a forging wherein the metal is worked throughout its entire mass.

2. In the manufacture of gun barrel forgings, the method which includes the steps of helically rolling a heated metallic workpiece over a mandrel to reduce the outside diameter thereof and to simultaneously pierce the same to provide a cylindrical forging having a bore of substantially the diameter desired in the finished article throughout the length thereof, then passing the workpiece over a mandrel between opposed spaced-apart rolls whereby the workpiece is helically rolled and tapered by varying the distance between the rolls while maintaining the bore substantially uniform, twisting said workpiece while it is helically rolled and maintaining the portion of the workpiece being worked under compression thereby producing a forging wherein the metal is worked throughout its entire mass.

3. In the manufacture of gun barrel forgings, the method including the steps as defined in claim 2, wherein the twisting of workpiece during the rolling thereof is in a direction opposite the direction of the subsequent helical rifling of the bore of the workpiece.

BRYANT BANNISTER.